

107

Patented Sept. 6, 1938

2,128,965

## UNITED STATES PATENT OFFICE

2,128,965

## ART OF MAKING LEATHERBOARD

Herman W. Richter, Bridgewater, Mass., assignor  
to George O. Jenkins Company, Bridgewater,  
Mass., a corporation of Massachusetts

No Drawing. Application March 31, 1936,  
Serial No. 71,926

## 6 Claims. (Cl. 8—2)

This invention relates to a method of making leatherboard which is also known as heeling board. These two terms are used interchangeably by persons skilled in the art to denote a material made from a furnish composed principally of leather scrap by board-making processes which involve disintegration in a beating engine, and subsequent formation into sheets or slabs on a wet machine. The product usually contains some 5 paper (generally not over 15%), introduced for process purposes and to impart certain desirable characteristics to the material, together with more or less leatherboard scrap. In this specification the term "leatherboard" will be used to 10 denote such a product without regard to the proportions of constituents, provided there is present sufficient leather to give it the desirable properties usually ascribed to the presence of leather fiber.

Leatherboard manufactured by the usual process 20 is of a rather dark, unattractive color, undoubtedly due to the presence of iron-tannate inks formed in the leatherboard during its fabrication by chemical reaction between the tannins present in the leather scrap and the iron of the 25 fabricating apparatus.

The most extensive commercial use of leatherboard is in the manufacture of heels for boots and shoes. Shoe heels made from the common dark colored leatherboard do not match the color of 30 either the uppers or the soles made of hide leather, and this fact has resulted in the use of leather for the manufacture of heels in many cases where leatherboard would have been used but for its dark color.

In my United States Patent No. 1,975,556, I disclosed a process for treating leatherboard by subjecting it to the bleaching action of certain chemicals, the preferred embodiment of which was 35 oxalic acid, to thereby remove the dark color of the iron-tannate inks either throughout the entire cross section thereof or in the outer cross-sectional zones. I have now discovered that by the use of solutions containing phosphoric acids such as orthophosphoric, pyrophosphoric, and meta-phosphoric the dark color of the iron-tannate 40 inks may be as effectively and more cheaply removed from the leatherboard, resulting in a leatherboard product having substantially the natural color of the leather fiber wherever it has been 45 treated with such an acid.

The primary object of this invention is to provide an improved method of manufacturing leatherboard which has the natural color of leather fiber.

Another object is to provide an improved

method of manufacturing leatherboard which has the natural color of leather fiber in any desired cross-sectional zone or zones.

The phosphoric acids may be applied to the furnish or to the leatherboard product in any of the following ways:—in the beater, in the vat, by dipping the leatherboard in the form of sheets or slabs in a solution of the acid, by spraying a solution of the acid upon one or both surfaces of sheets or slabs of the leatherboard, or by spraying a solution of the acid upon one or more layers of the leatherboard as it is being built up on the wet machine.

As illustrative of the application by dipping, a sheet of leatherboard is dipped in an aqueous 15 solution of orthophosphoric acid of between 1% and 6% concentration. A 3% concentration gives a pale colored product of substantially the natural color of the outer cross-sectional areas of a cut section of hide leather. Less concentrated 20 solutions do not produce a leatherboard of such pale color.

The required dipping time depends upon the thickness and density of the leatherboard and also upon the final cross-sectional color effect which is 25 desired. In making a product in which the dark color of the iron-tannate inks is removed from its entire cross-section it is necessary to keep the board immersed in the solution long enough to permit the solution to penetrate the entire thickness of the board and thus allow it to come in contact with the iron-tannate inks throughout its entire thickness. In the case of boards of average thickness and density, a dipping time of 30 five minutes or more is sufficient. In producing 35 a product which has pale colored outer cross-sectional zones and a dark colored center cross-sectional zone or core, the leatherboard is dipped in the solution only a sufficient time to allow penetration into the outer cross-sectional zones, usually between thirty seconds and five minutes for 40 boards of average thickness and density. The center cross-sectional zone into which the solution does not penetrate thus retains its original dark color, and in the outer cross-sectional zones 45 the dark color is removed by the acid solution.

A test run may be made with a sample taken from the leatherboard to be treated, to determine the proper dipping time to produce the desired 50 cross-sectional color effect.

By means of suitable concentrations and suitable dipping times in the use of the other phosphoric acids, I have found it possible to produce results substantially similar to those produced with orthophosphoric acid.

5

10

20

25

30

35

40

45

50

55

So far as I have been able to determine from a search of the literature I am the first to use phosphoric acids to eliminate or remove the dark color due to iron-tannate inks and to thereby liberate the natural color of the leather fiber. These acids are much cheaper than oxalic acid, the preferred embodiment of my prior patent, and they produce as good, if not better, color effects in the final product.

10 It is to be understood that the foregoing disclosure is merely illustrative of my invention and is not to unduly restrict the scope of the following claims. It is also to be understood that my invention is not dependent upon any explanations or theories which I have set forth as descriptive of the actions involved, nor dependent upon the soundness or accuracy of any theoretical statements so advanced.

I claim:

1. The method of making leatherboard which comprises subjecting leatherboard containing iron-tannate inks to the action of a solution containing a phosphoric acid. 5
2. The method as defined in claim 1, wherein the phosphoric acid solution has a concentration of from 1% to 6%.
3. The method as defined in claim 1, wherein the phosphoric acid solution has a concentration 10 of about 3%.
4. The method as defined in claim 1, wherein the phosphoric acid is orthophosphoric acid.
5. The method as defined in claim 1, wherein the phosphoric acid is metaphosphoric acid. 15
6. The method as defined in claim 1, wherein the phosphoric acid is pyrophosphoric acid.

HERMAN W. RICHTER.